

1

3,044,955

**ELECTRICAL INSULATING OILS**

Wilhelmus C. de Groot and Hubertus N. H. de Haan, both of Amsterdam, Netherlands, and Ralph W. van den Bosch, Sevenoaks, England, assignors to Shell Oil Company, a corporation of Delaware  
No Drawing. Filed May 27, 1959, Ser. No. 816,973  
Claims priority, application Great Britain June 3, 1958  
1 Claim. (Cl. 208—212)

This invention relates to improved insulating oils. More particularly, it relates to a process for preparing electrical insulating oils which are oxidation stable, non-sludging, and resistant to gassing.

Certain hydrocarbon oils are used in electrical applications such as transformers, circuit breakers, and high voltage cables because of their high dielectric strength. However, because of the susceptibility of such hydrocarbons to oxidation, which results in the formation of sludge and acid, hydrocarbon oils for electrical applications must be carefully refined. The high electrical stress to which insulating oils are subjected also tends to decompose the oil thus producing sludge and gaseous products which may cause serious damage and failure of the apparatus in which they are used. The presence of aromatic hydrocarbons in the oil tends to inhibit such decomposition (gassing), but they have an adverse effect in that they increase oxidative sludging. The principal detrimental effect of sludging and acid formation and gassing is to raise the dielectric constant and power factor. In addition, substantial corrosion of electrical components is often caused by the acids formed by sludging and gassing. Drastic refining of highly aromatic oils to produce more stable electrical insulating oils results in poor yields, which are generally as low as 45-55% by weight, calculated on the basis of the starting material.

Mineral oils having a viscosity of between about 1 and 9 degrees Engler at 20° C. (generally between 3 and 5 degrees Engler at 20° C.) are generally used as dielectric oils in electrical equipment.

For preparing electrical insulating oils, the starting material is usually a straight-run mineral oil distillate of the above viscosity. Usual refining methods are extraction with a selective solvent for the aromatic components of the oil (e.g., liquid sulfur dioxide or furfural) and treatment of the raffinate with concentrated sulfuric acid or oleum. Combinations of these treatments may be used and they are usually followed by a finishing treatment with a solid adsorbent, such as clay. If desired, the oils thus obtained may also be mixed with a small amount of an extract obtained by selective extraction after this has also been treated with concentrated sulfuric acid or oleum. In this connection reference may be made to British specifications 589,149 and 589,150. These usual refining methods have the disadvantages that they are rather costly and that considerable amounts of the oil are lost, as mentioned above.

Desulfurization by selective hydrogenation (frequently termed hydrofining or hydrodesulfurization) is a refining method which is cheap and wherein only small amounts of the oil are lost. It has already been proposed to apply this refining method in the preparation of electrical insulating oils. From *Brennstoffchemie*, 36, 218 (1955), it is known to prepare an electrical insulating oil by first removing the sulfur completely from a shale oil by hydrogenation and then treating the hydrogenated oil with sulfuric acid and bleaching earth. From *The Oil and Gas Journal*, 53, 84 (1954) it is known to prepare an electrical insulating oil by extracting a distillate obtained from a Tia Juana crude oil with liquid sulfur dioxide, so as to obtain a raffinate having a sulfur content of

2

0.42% by weight and then hydrogenating the raffinate so as to obtain an oil having a sulfur content of 0.06% by weight. Thus, in these known processes the hydrogenation is still combined with an extraction or an acid treatment.

It is therefore an object of this invention to provide a process for the production of electrical insulating oils with satisfactory properties in a simple and inexpensive manner and in high yields. It is a further object of this invention to provide a process for the production of insulating oils having excellent oxidation stability and very low gassing tendencies. Other objects will be apparent from the detailed description of the process of this invention which comprises a particular combination of selective hydrodesulfurization of mineral oil distillate and treatment with a solid adsorbent.

By selective hydrodesulfurization is here meant a hydrogenation under conditions in which the non-hydrocarbons present in the oil (viz. the compounds which in addition to carbon and hydrogen contain other elements, such as sulfur or oxygen) are hydrogenated, but the hydrocarbons remain essentially unaffected (so that, for example, there is virtually no cracking of the oil or hydrogenation of aromatics present in the oil). Several methods are already known (see, for example, "Erdol and Kohle," 6, 616-619 (1953)) for selectively hydrogenating oils in this way. The oil may be in either the gas or the liquid phase during the hydrogenation, a very suitable method being trickle phase hydrogenation, wherein a very thin layer of the oil is allowed to flow over a bed of a catalyst. In general the selective hydrogenation is carried out at a temperature of 300-400° C., a pressure of 10-200 kg. per sq. cm., a gas discharge rate of 50-5,000 liters per kg. of oil and a flow rate of the oil of 0.3-3 kg. per liter of catalyst per hour. Suitable catalysts are oxygen or sulfur containing compounds such as oxides and sulfides of metals of groups VI and VIII of the periodic table. Especially preferred are cobalt oxide, molybdenum oxide, tungsten sulfide and nickel sulfide. The catalysts are preferably such compounds supported on a carrier, such as active carbon, fuller's earth, kieselguhr, silica or alumina, e.g. in the form of bauxite, pumice or burnt clay. Very suitable catalysts are described in British specification 657,400 and of these the catalysts comprising cobalt oxide and molybdenum oxide on an aluminum oxide-containing carrier, such as bauxite, are particularly preferred. Of the latter class of catalysts, the catalyst referred to as high cobalt catalysts which contain cobalt and molybdenum in an atomic ratio between about 0.7 and 0.8, are particularly effective. The catalysts may be used in the form of cylindrical tablets measuring, for example, 5 x 5 or 3 x 3 mm. Suitable hydrogenation methods are described for example in British specifications Nos. 657,521, 665,575 and 699,455.

An important feature of the invention is that the selective hydrodesulfurization should be carried out so that the oil is not completely desulfurized. Generally, the hydrogenated oil should still contain at least 0.05% by weight of sulfur and in most cases not more than 95% of the sulfur originally present in the oil should be removed. On the other hand, the sulfur content of the hydrogenated oil should not be too high and should generally not exceed 0.6% by weight. In most cases at least 60% of the sulfur originally present in the oil should be removed. Removal of about 70-90% of the sulfur originally present is preferred. The exact mechanism by which the incomplete hydrodesulfurization contributes so unexpectedly to the stability of the insulating oils is not fully understood. The sulfur compounds remaining in the oil after the hydrotreating step are, of course, more

hydrogenation resistant and of different average composition and configuration than those which are removed. Therefore, because of the partial removal of other sulfur compounds, and because of the different composition of the residual sulfur compounds, they appear to exhibit a unique inhibitory effect which is not realized from an oil of like sulfur content which has not been hydrodesulfurized or which has been desulfurized by other means.

Within the above limits, the optimum extent of desulfurization depends on the specification which the finished oil must satisfy. In this connection it should be noted that various methods for testing the oxidation stability of electrical insulating oils exist. However, the properties of the oils produced according to the process of this invention as described herein are evaluated by the specification and tests of the British Standards Institution (BSI). Details of the BSI test, as it is hereinafter referred to, are found in test B.S. 148:1951 of the British Standards Institution.

When desulfurized to the extent indicated above, an oil will be obtained which satisfies at least one of these specifications and can, therefore, be considered to be suitable for use as an electrical insulating oil. Hydrogenation to a sulfur content of 0.15-0.35% by weight (still more preferably 0.20-0.30% by weight) is very suitable, since then from various starting materials an insulating oil can be obtained which satisfies more than one specification at the same time, which is of advantage to the manufacturer from the point of view of economy of production.

In the selective hydrogenation, hydrogen sulfide is formed from the sulfur compounds present in the oil. A part of the hydrogen sulfide formed dissolves in the oil, and this should be removed from the oil. This can be effected, for example, by washing the oil with a caustic alkali solution, but it is most simply carried out by blowing through the oil an inert gas such as nitrogen, if desired, at elevated temperature or by stripping with steam.

Electrical insulating oils are often required to have a flash point which is not below a certain temperature. As a result of the selective hydrogenation the initial boiling point of the oil is somewhat reduced. This causes a lowering of the flash point of the oil. As a result the flash point of the final insulating oil may not satisfy the flash point requirement. If this is the case, the low boiling components should be removed from the oil. This can be done in a simple way by means of steam-stripping or distillation, preferably under reduced pressure, until the residue has the desired flash point. A Pensky-Martens closed cup (PMCC) flash point of at least 120° C. is desirable, and a PMCC flash point of at least 146° C. is preferred.

Finally, in the process of the invention, the oil is treated with a solid adsorbent such as fuller's earths and activated clays. Suitable adsorbents, are, for example, fuller's earths of the attapulgite and montmorillonitic types and acid activated clays such as bentonite, bauxite, and alumina. Small quantities of alkaline material such as lime may be added to the adsorbent. If desired, the oil may be heated during the treatment (for example, to a temperature of about 50-100° C.), and an inert gas such as nitrogen passed through the oil. The quantity of adsorbent used generally lies between 0.5 and 30% by weight, preferably between 1 and 5% by weight, calculated on the oil treated.

The process of the invention is generally applicable to mineral oil fractions having a viscosity between about 1 and 9 degrees Engler at 20° C., i.e. light lubricating oil distillates, such as spindle oils. In most cases a distillate boiling in the range of from 300 to 500° C. is used as the starting material. Of course, the starting material should be so selected, that after desulfurization to the prescribed extent the desired sulfur content can be attained. The process of the invention is of particular

advantage for starting materials having a relatively high sulfur content, i.e. oils having a sulfur content of at least 1% by weight, and particularly those having a sulfur content of at least 1.5% by weight.

It is not necessary to separate first the desired light lubricating oil distillate from a mineral oil and then to hydrogenate the separated distillate and to treat it with a solid adsorbent. It is also possible to start from a fraction which in addition to the desired light lubricating oil contains heavier components, such as heavier lubricating oils, and/or lighter components, such as gasoline, kerosene or gas oil. Such a fraction may be selectively hydrogenated and the desired light lubricating oil separated from it after the hydrogenation by distillation. In this distillation the flash point of the separated light lubricating oil distillate fraction may be adjusted at the same time to the desired value.

The aromatic content of the oil is reduced very little during the selective hydrogenation for the reasons stated above. Also during the treatment with a solid adsorbent no substantial reduction of the aromatic content of the oil occurs. A high aromatic content of an electrical insulating oil has a favorable effect on its gassing characteristics, so that the process of the invention provides an excellent means for preparing insulating oils with good characteristics. This becomes particularly apparent when starting materials having a relatively high aromatic content are used, e.g. oils having an aromatic content of at least 30% by weight and particularly those having an aromatic content of at least 40% by weight.

When, in this specification, reference is made to an aromatic content of an oil, the aromatic content is that determined by percolation over silica gel as described in "Journal of the Institute of Petroleum," 36, 89-104 (1950).

The following examples illustrate the process of the invention.

#### EXAMPLE I

##### Run A

40 The starting material was a spindle oil obtained by distilling a naphthenic crude oil. This distillate had the following properties:

Viscosity \_\_\_\_\_ 5.5 degrees Engler at 20° C.  
45 Flash point (Pensky-Martens, closed cup) \_\_\_\_\_ 156° C.  
Sulfur content \_\_\_\_\_ 1.76% by weight.  
Aromatic content \_\_\_\_\_ 50% by weight.

50 This oil was selectively hydrodesulfurized by allowing it to flow in a thin layer over a catalyst bed (cobalt oxide and molybdenum oxide supported on bauxite; 4% by weight of cobalt oxide and 10% by weight of molybdenum oxide calculated on total catalyst; atomic ratio Co:Mo=0.768) in the form of cylindrical tablets measuring 3 x 3 mm., under the following conditions:

Temperature, ° C. \_\_\_\_\_ 375  
Pressure, kg./sq. cm. \_\_\_\_\_ 50  
Flow rate of the oil, kg./liter catalyst/hour. \_\_\_\_\_ 1.9  
60 Gas discharge rate, liter kg. oil. \_\_\_\_\_ 200

Approximately 2% by weight of the oil was lost during the selective hydrogenation.

65 The oil was stripped with steam in order to remove the hydrogen sulfide and the lightest components. Approximately 8% by weight of the oil was removed during this treatment. The remaining oil had a flash point of 148° C., a sulfur content of 0.25% by weight and an aromatic content of 45% by weight.

Finally the oil was treated at a temperature of 75° C. 70 with 3% by weight of Filtrol for 1/2 hour while nitrogen was passed through it. The yield of final electrical insulating oil was 88% by weight, calculated on the total amount of starting material.

The oxidation stability of the final oil was determined 75 in the B.S.I. test (B.S. 148/1951). According to the

specification, after the conclusion of the test the limit of sludge formation in the oil should be 1.2% by weight and the maximum acid number of the oil 2.5. The oil satisfied this specification: after the test the oil had a sludge value of 1.1% by weight and an acid number of 0.8.

The gassing characteristics of the final oil were evaluated in the modified Pirelli apparatus (Journal of the Institute of Petroleum, 35, No. 311, pp. 735-754) at a temperature of 50° C. under a hydrogen atmosphere and a voltage of 10 kv. The amount of hydrogen is measured which the oil absorbs or evolves under these conditions in the course of time. The hydrogen absorption or hydrogen evolution expressed in mm. of oil pressure is plotted in a graph as a function of the time and the slope of the line thus obtained determines the gassing coefficient of the oil. For the present oil this coefficient was found to have the very favorable value of -8, which means that the oil is very strongly gas absorbing.

In the following runs some comparative tests are described.

#### Run B

The procedure of Run A was repeated, except that the Filtrol treatment of the oil was omitted. In the B.S.I. test the oil had a sludge value of 2.4% by weight and an acid number of 2.0.

#### Run C

The same starting material used in Run A was hydrogenated and stripped with steam as described for Run A. Then the oil was treated with 2% by weight of 96% sulfuric acid for ½ hour at a temperature of 20° C. The acid sludge was then allowed to deposit and was separated off. Finally the oil was treated with 3% by weight of Filtrol, to which 0.2% by weight of lime had been added (the percentages are calculated on the quantity of oil treated), at 75° C. for ½ hour while nitrogen was passed through it. In the B.S.I. test the final oil had a sludge value of 1.63% by weight and an acid number of 1.3.

#### Run D

An electrical insulating oil satisfying the B.S.I. test was prepared by a conventional method from the same starting material as was used in Run A.

The oil was first extracted with liquid sulfur dioxide (ratio by volume of oil:SO<sub>2</sub>=1:1.3. The raffinate thus obtained was treated with 10% by weight of oleum (containing 17% by weight of dissolved SO<sub>3</sub>) for ½ hour at a temperature of 20° C. The acid sludge was then allowed to deposit and was separated off. The oil was washed with a 4% solution of NaOH in 40% aqueous alcohol and subsequently with dilute alcohol and water. Finally the oil was treated at 75° C. with 3% by weight of Filtrol for ½ hour while nitrogen was passed through it. The yield of final electrical insulating oil was 55% by weight. In the B.S.I. test the oil had a sludge value of 0.84% by weight and an acid number of 1.4. The gassing coefficient of the oil was positive.

#### Run E

The same starting material as used in Run A was extracted with liquid sulfur dioxide (ratio by volume of oil:SO<sub>2</sub>=1:2) so as to obtain a raffinate having a sulfur content of 0.48% by weight. The raffinate was then selectively hydrogenated as described in Example I, with the exception that the reaction conditions were so modified that the oil (after steam-stripping) had a sulfur content of 0.04% by weight. The oil was finished by treatment with Filtrol as described in Example I. In the B.S.I. test the oil had a sludge value of 1.65% by weight and an acid number of 2.7.

The oxidation stability of oils prepared according to the process of the invention (to be referred to herein-after as "oils of type A") can be improved by the addition

of mineral oil fractions having a lower aromatic content (to be referred to hereinafter as "oils of type B"). These are generally used in a minor proportion. For example, 90-60 parts by weight of an oil of type A may be blended with 10-40 parts by weight of an oil of type B. It is clear that this possibility is particularly of importance for oils of type A having a high aromatic content. Of course, the sulfur content of the oil of type B should not be such that the sulfur content of the final mixture becomes unduly high. Generally the sulfur content of the final mixture should not be above 0.6% by weight.

The oil of type B is preferably obtained from the same starting material as the oil of type A to result in an especially suitable electrical insulating oil in accordance with the invention.

Oils of type B may be obtained by extracting an oil in a known manner with a selective solvent for the aromatic components of the oil, e.g. liquid sulfur dioxide or furfural. The oil of type B may also be subjected to other refining treatments, such as treatment with concentrated sulfuric acid or oleum or selective hydrogenation. Generally the oil of type B is also subjected to a finishing treatment with a solid adsorbent. This finishing treatment may be carried out in the same way as described above in connection with the preparation of the oil of type A. The finishing treatment may be carried out either on the oils of type A and B separately, or after blending.

If during the preparation of the oil of type B extraction with concentrated sulfuric acid or oleum is applied, this treatment may be carried out in any known manner. For instance, concentrated sulfuric acid (80-100%) or oleum (up to 30% by weight dissolved SO<sub>3</sub>) may be used in amounts of from 5-30% by weight, calculated on the oil treated, as temperatures varying from 0° to 75° C. and contact times from 5 sec. to one hour. The extraction can be carried out in one or more stages and either batchwise or continuously. In batchwise refining the treatment temperature is preferably approximately 25° C., and in continuous refining preferably approximately 60° C. After the extraction with concentrated sulfuric acid or oleum, the acid sludge is removed from the oil. The oil may then be neutralized by treatment with an alkaline material, such as an aqueous or alcoholic solution of NaOH, which may be followed by washing with water and/or alcohol. Alternatively, an alkaline material, such as lime, may be added to the solid adsorbent with which the oil is finished.

According to a particular aspect of the invention, the oil of type B is prepared by extracting an oil with a selective solvent for the aromatic components of the oil followed by subjecting the raffinate thus obtained to a treatment with concentrated sulfuric acid or oleum and a finishing treatment with a solid adsorbent. This is illustrated by the following example.

#### EXAMPLE II

An oil of type B was prepared from a portion of the same starting material as used in Example I. This portion of the starting material was extracted with liquid sulfur dioxide, so as to obtain a raffinate having an aromatic content of 9% by weight. This raffinate was treated with oleum, neutralized and finished with Filtrol as in Run D of Example I.

Twenty parts by weight of this oil (type B) were mixed with 80 parts by weight of the oil (type A) prepared according to Example I. In the B.S.I. test the final blend had a sludge value of 0.65% by weight and an acid number of 0.4. The gassing coefficient of the final blend was -4. The yield of finished electrical insulating oil was 74% by weight, calculated on the total amount of starting material.

According to another aspect of the invention, the oil of type B is prepared by selectively hydrogenating an oil

as described above in connection with the preparation of the oil of type A, extracting the hydrogenated oil with a selective solvent for the aromatic components of the oil and subjecting the raffinate thus obtained to a finishing treatment with a solid adsorbent. Particularly, an insulating oil may be prepared as follows. The starting material is selectively hydrogenated and the hydrogenated oil is divided into two parts. One part is treated with a solid adsorbent so as to obtain an oil of type A. The other part is extracted with a solvent selective to aromatics and the raffinate thus obtained is treated with a solid adsorbent so as to obtain an oil of type B. Finally the oils of type A and B are mixed. Instead of treating the two oils separately with a solid adsorbent, they may also be mixed before being treated with a solid adsorbent and the mixture treated with a solid adsorbent. Preferably a proportion of at least 10 but not more than about 60% by weight of the hydrogenated oil is extracted. The conditions of extraction are preferably such as to give a raffinate yield of at least 70% by weight of the extracted portion of the hydrogenated oil. The degree of extraction of a 60% proportion of hydrogenated oil would thus be about 18% of the whole hydrogenated oil. In preparing oils of type B, whether from the hydrodesulfurized or untreated starting material, the degree of extraction should be limited to not more than 20% by weight of the starting material. The raffinate and unextracted hydrogenated oil after blending therefore comprises at least 80% by weight of the original hydrogenated oil. The following example illustrates this embodiment of the invention.

### EXAMPLE III

The same starting material as was used in Example I was selectively hydrogenated and steam stripped as described in Example I. Several portions of the hydrogenated oil thus obtained were extracted with liquid sulfur dioxide under the conditions mentioned in the following table.

| Run No. | Solvent ratio, vol./vol. | Extraction temperature, °C. | Raffinate yield |             |
|---------|--------------------------|-----------------------------|-----------------|-------------|
|         |                          |                             | Percent vol.    | Percent wt. |
| F1..... | 0.8:1                    | 32-38                       | 84.3            | 82.7        |
| F2..... | 1.0:1                    | 32-38                       | 79.0            | 77.2        |
| F3..... | 1.2:1                    | 32-38                       | 78.0            | 76.1        |
| F4..... | 1.5:1                    | 32-38                       | 74.2            | 72.1        |
| F5..... | 1.8:1                    | 32-38                       | 72.3            | 70.0        |

The raffinates thus obtained were mixed in varying proportions with the unextracted hydrogenated oil and the mixtures were finished by treatment with Filtral as described in Example I. The blending proportions as well as the B.S.I. test results of the finished electrical insulating oils are given in the following table.

| 5       | Unextracted hydrogenated oil, amount, percent wt. | Raffinate           |        | B.S.I. test         |                        |
|---------|---------------------------------------------------|---------------------|--------|---------------------|------------------------|
|         |                                                   | Amount, percent wt. | Number | Sludge, percent wt. | Acid value, mg. KOH/g. |
| 60..... | 40                                                | 1                   | 0.7    | 0.6                 |                        |
| 60..... | 40                                                | 2                   | 0.7    | 0.7                 |                        |
| 60..... | 40                                                | 3                   | 0.8    | 0.8                 |                        |
| 60..... | 40                                                | 4                   | 0.5    | 0.5                 |                        |
| 60..... | 40                                                | 5                   | 0.7    | 0.8                 |                        |
| 80..... | 20                                                | 3                   | 0.9    | 0.6                 |                        |
| 80..... | 20                                                | 4                   | 0.8    | 0.6                 |                        |

15 All these blends were strongly gas-absorbing, viz., they exhibited a negative gassing coefficient.

If desired, small quantities (e.g. between 0.01 and 1% by weight) of anti-oxidants may be added to the insulating oils prepared according to the invention. As such, 20 alkyl phenols, such as 2,6-di-tert.butyl-4-methyl phenol, are particularly suitable. In this connection it should be observed that the insulating oils of the invention usually have a good inhibitor susceptibility.

We claim as our invention:

25 A process for the production of an oxidation stable non-gassing insulating oil from a sulfur-containing mineral lubricating oil mixture which also contains aromatics and boils within the range from about 300 to about 500° C. consisting essentially of the steps of (1) selectively hydrodesulfurizing said mixture without appreciable conversion of hydrocarbons therein to reduce the sulfur content by at least 70% but by not more than about 90% by weight, (2) separating from the hydrodesulfurized mixture by means of fractional distillation a light lubricating oil fraction boiling from about 300 to about 500° 30 C. having a viscosity at 20° C. of from about 1 to about 9 degrees Engler and having a Pensky-Martens closed cup flash point of at least 120° C., (3) separating from the light lubricating oil fraction a portion comprising at least 10% but not more than 60% by volume thereof, (4) extracting the separated portion of light lubricating oil fraction by means of an aromatics-selective solvent to a depth such that the aromatics-containing extract does not exceed 20% by volume of the total light lubricating oil fraction, (5) blending the raffinate from the extraction 40 step with the unextracted portion of the separated light lubricating oil fraction, and (6) treating the blended mixture of extracted and unextracted light lubricating oil fraction with between 0.5 and 30% by weight, based on the blended mixture, of a solid adsorbent.

### References Cited in the file of this patent

#### UNITED STATES PATENTS

2,865,849 Van Loom et al. ..... Dec. 23, 1958  
55 2,944,012 Thompson ..... July 5, 1960